# EUROPEAN PATENT SPECIFICATION

(11) **EP 1 984 527 B1**
(45) Date of publication and mention of the grant of the patent: **06.11.2013**
(21) Application number: 06818001.7
(22) Date of filing: 06.12.2006
(51) Int. Cl.: C21D 9/08, C21D 8/02, C21D 8/04, C22C 38/02, C22C 38/04

(54) **METHOD OF PRODUCTION OF HIGH-STRENGTH LOW-ALLOYED STEEL PIPES**
VERFAHREN ZUR HERSTELLUNG VON ROHREN AUS NIEDRIG LEGIERTEM STAHL MIT HOHER FESTIGKEIT
PROCEDE DE PRODUCTION DE CONDUITES EN ACIER FAIBLEMENT ALLIE A HAUTE RESISTANCE

(30) Priority: 06.12.2005 CZ 20050756
(43) Date of publication of application: 29.10.2008
(73) Proprietor: Comtes FHT a.s., 334 41 Dobrany (CZ)
(72) Inventor: NOVY, Zbysek, 330 Tlucna (CZ); KRAUS, Libor, 330 22 Zbuch (CZ); ZRNIK, Jozef, 04 001 Kosice (SK); NEMECEK, Stanislav, 301 62 Pizen (CZ)
(74) Representative: Langrova, Irena
(86) International application number: PCT/CZ2006/000086
(87) International publication number: WO 2007/065380

(56) References cited:
- JP-A- 5 096 323
- JP-A- 7 246 481
- JP-A- 61 056 233
- JP-A- 63 213 620
- US-A1- 2003 051 782
- US-A1- 2003 116 238
- M.A. MALEQUE, Y.M. POON, H.H. MASJUKI: "The effect of intercritical heat treatment on the mechanical properties of AlSi 3115 steel" JOURNAL OF MATERIALS PROCESSING TECHNOLOGY, vol. 153-154, 10 November 2004 (2004-11-10), pages 482-487, XP002481940 NL

## Description

### Field of the Invention

The invention concerns a method of production of high-strength low-alloyed steel pipes by drawing, extrusion, rolling or by combination of these steps from steels with controlled multi-phase microstructures.

### Prior Art

According to similar solutions, which have been known up to this day, the object of the invention as described in the document no. US 2003116238 concerns high strength steel pipes with excellent material formability produced for hydroforming and similar forming processes. Chemical composition of the pipe material is listed in weight per cent: 0.0005 - 0.30 % C, 0.001 - 2.0 % Si, 0.01 - 3.0 % Mn and appropriate amounts of alloying elements if needed. The balance consists of iron and unavoidable amount of additional elements.
However, the solution as described in this document does not specify the technological process which would ensure formation of required microstructure in the material and the required propertis.

JP7246481 discloses a process of producing a high quality large diameter clad steel tube by hot rolling and controlled cooling. The slab is heated to 1100-1250°C, rolled at 850-10000° C at a total draft of 5 or more, cooled with air for 60-200 sec. and cooled from 800°C or above to 600°C or below at a cooling speed of 5-40°C/sec.

According to the document no. US 2003051782, the steel pipe composition is as follows: 0.05 - 0.3 % C, 1.8 - 4 % Mn. The material with silicon and aluminium is rolled to reduce its diameter, where the overall diameter reduction is no less than 20% and the finish rolling temperature in diameter-reduction rolling is no higher than 800°C. The microstructure obtained in this fashion consisting of martensite and/or bainite or even ferrite was achieved as a product of deformed austenite transformation.
The solution consists in a material for pipes with tensile strength above 1,000 MPa and excellent three-point bending properties. The chemical composition of the steel pipes as described in this document may additionally contain at least one of the following group of elements: Cu, Ni, Cr and Mo or at least one of the following group of elements: Nb, V, Ti and B or at least one element of the group of rare earth metals and Ca.
However, the solution as described in this document does not specify the technological process, which would guarantee the formation of required microstructure and the required propertis.

### Summary of the Invention

A method of production of high-strength low-alloyed steel pipes, whereby the pipes are made by extrusion, rolling or by a combination of these processes and the pipes are made from a steel with multi-phase microstructure. The chemical composition of the material is as follows:
0.10 to 0.45 wt. % C, 1.2 to 2.5 wt. % Mn, 1.2 to 2.5 wt. % Si, the balance consisting of Fe and minute amounts of trace elements. The material also consists of impurities in the amount of up to 0.03 wt. % S, up to 0.03 wt. % P, up to 0.08 wt. % Cu, up to 0.08 wt. % Al and preferably containing microalloying elements Nb, V, Ti.
The production process is based on thermomechanical treatment and/or intercritical heat treatment, where the thermomechanical treatment consists in hot rolling and subsequent cooling or hot extrusion and subsequent cooling.

The first stage of production of pipes is the hot rolling process or hot extrusion process,
where the temperature at the end of rolling or extrusion is between 600 and 1,000°C, the entire process ends with controlled cooling, where the time period in the temperature range between 700 and 450°C is no more than 50 seconds and the period in the range of 450 to 350°C is at least 200 sec.

Another alternative solution consists of the following sequence: hot rolling or hot extrusion, cooling and intercritical heat treatment with the maximum temperature between 770 and 850°C. The hold at this temperature is followed by controlled cooling, as specified in the basic procedure.

There is another alternative solution, where the hot rolling or hot extrusion process is followed by cooling and drawing or forming by internal pressure or pipe bending. It is then followed by intercritical heat treatment with the maximum temperature between 770 and 850°C. The hold at this temperature is followed by controlled cooling, as specified in the basic procedure.

The advantage of this solution lies in the possibility to obtain high-strength pipes with high plasticity level required for cold forming, e.g. drawing and/or bending and/or hydroforming (forming with internal pressure). With this solution, it is possible to achieve the required multi-phase microstructure with excellent properties either by means of thermomechanical treatment or by intercritical heat treatment.
The available choice between the above alternatives represents another advantage. It is because in some plants it is not possible to perform thermomechanical treatment. Moreover, in some applications, drawing has to be carried out before the processing for the required microstructure. In the latter case, the microstructure development can be achieved with the intercritical heat treatment.

### Examples of the Ivention Embodiment

### Example 1

A steel consisting of 0.03 wt. % S max., 0.03 % P max., 0.08 % Cu max., 0.08 % Al max., 0.10 to 0.45 wt. % C, 1.2 to 2,5 wt. % Mn, 1.2 to 2,5 wt. % Si, with the balance of Fe and minute amounts of trace elements and preferably containing microalloying elements: Nb, V, Ti, has been used for making high-strength low-alloyed steel pipes,
The pipes were made from steels with multiphase microstructures by means of rolling, controlled cooling and subsequent drawing.
In this example, thermomechanical treatment has been used for production of pipes. This process involved hot rolling with finishing temperature between 800 and 900°C.
Next process was controlled cooling with 25 sec delay in the temperature range of 700 to 450°C and 300 sec delay in the 450 - 350°C temperature range.
The processing is concluded with a single-pass drawing, i.e. without interstage annealing. This fact (preferable advantage) is a result of high plasticity of material that has been achieved owing to the multi-phase structure of the steel. The controlled multi-phase structure of the material with the required amount of plasticity has been achieved during the thermomechanical treatment and controlled cooling sequence.

### Example 2

A steel consisting of 0.03 wt. % S max., 0.03 wt. % P max., 0.08 wt. % Cu max., 0.08 wt. % Al max., 0.10 to 0.45 wt. % C, 1.2 to 2,5 wt. % Mn, 1.2 to 2,5 wt. % Si, with the balance of Fe and minute amounts of trace elements and preferably containing microalloying elements: Nb, V, Ti, has been used for making high-strength low-alloyed steel pipes.
The pipes were made from steels with multiphase microstructures by means of rolling, drawing and intercritical heat treatment.
In this example, the procedure used for the pipe production consisted in the procedure involving the sequence of hot rolling or hot extrusion, cooling, drawing and intercritical heat treatment with heating to 800°C.
Upon soaking at this temperature, controlled cooling is applied with delay in the temperature range of 700 to 450°C of 15 sec and the delay in the temperature range of 450 to 350°C is 400 sec.
A pipe produced in this fashion can be used for forming by internal pressure, which requires that the material shows high plasticity. The controlled multi-phase structure of the material with the required amount of plasticity has been achieved by the intercritical heat treatment and controlled cooling sequence.

### Industrial Utility

The proposed solution is practically usable in production of transport vehicles, in particular cars, buses and rail vehicles.

## Claims

1. A method of production of high-strength low-alloyed steel pipes from a material consisting of impurities in the amounts of 0.03 wt. % S max., 0.03 % P max., 0.08 % Cu max., 0.08 % Al max. and also consisting of 0.10 to 0.45 wt. % C, 1.2 to 2.5 wt. % Mn, 1.2 to 2.5 wt. % Si with the balance of Fe and minute amounts of trace elements and preferably containing microalloying elements Nb, V, Ti where the pipes are produced by drawing, extrusion, rolling or combination of these processes from steels with multi-phase microstructure, **characterized in that** the manufacturing procedure consists of thermomechanical treatment and/or intercritical heat treatment, where the pipes are produced by hot rolling or hot extrusion with finish forming temperature between 600 and 1,000 °C and subsequent controlled cooling with delay of maximum 50 sec in the temperature range of 700 to 450°C and the delay of at least 120 sec in the temperature range of 450 to 350 °C.

2. A method of production of high-strength low-alloyed steel pipes of claim 1,
**characterized in that** the hot rolling or hot extrusion process is followed by the following sequence: a cooling process, intercritical heat treatment at the maximum temperature between 770 and 850 °C, upon soaking at this temperature before the step of controlled cooling.

3. A method of production of high-strength low-alloyed steel pipes of claim 2,
**characterized in that** the hot rolling or hot extrusion process is followed by a cooling process and the production is concluded with drawing and/or forming by internal pressure and/or bending.

## Patentansprüche

1. Methode der Herstellung der hochfesten niedriglegierten Stahlrohren aus dem den Schmutz in Mengen von höchstens 0,03 Gew.-Prozent von S, höchstens 0,03 Gew.-Prozent von P, höchstens 0,08 Gew.-Prozent von Cu, höchstens 0,08 Gew.-Prozent von Al und auch 0,10 bis 0,45 Gew.-Prozent von C, 1,2 bis 2,5 Gew.-Prozent von Mn, 1,2 bis 2,5 Gew.-Prozent von Si mit Rest von Fe enthaltenden Material, das geringe Spurelementmengen und vorzugsweise auch mikrolegierende Elemente Nb, V, Ti enthält, wobei die Rohre durch Ziehen, Stoßräumen, Walzen oder Kombinationen dieser Prozesse aus Stähle mit multiphasiger Mikrostruktur erzeugt werden,
**dadurch gekennzeichnet, dass** die Herstellungsprozedur aus thermomechanischer Behandlung und/oder interkritischer Wärmebehandlung besteht, wo die Rohre durch Warmwalzen oder Strangpressen mit Endformierungstemperatur zwischen 600 und 1.000 °C
und nachfolgender gesteuerter Kühlung mit Verzögerung von höchstens 50 Sek. im Temperaturbereich von 700 bis 450 °C und Verzögerung von mindestens 120 Sek. im Temperaturbereich von 450 bis 350 °C hergestellt werden.

2. Methode der Herstellung der hochfesten niedriglegierten Stahlrohren nach dem Anspruch 1,
**dadurch gekennzeichnet, dass** nach dem Warmwalzen- oder Warmstrangpressenprozess folgende Reihenfolge nachkommt: der Kühlungsprozess, die interkritische Wärmebehandlung auf der Höchsttemperatur zwischen 770 und 850°C mit Anlassen auf dieser Temperatur vor dem gesteuerten Kühlungsschritt.

3. Methode der Herstellung der hochfesten niedriglegierten Stahlrohren nach dem Anspruch 2,
**dadurch gekennzeichnet, dass** nach dem Warmwalzen- oder Warmstrangpressenprozess der Kühlungsvorgang folgt und die Herstellung durch Ziehen und/oder Innendruckformung und/oder Biegen beendet wird.

## Revendications

1. Méthode de la production des tuyaux d'acier à haut rigidité et à basse alliage de matériel contenant des impuretés en quantités de 0,03 pour cent de masse de S au maximum, 0,03 pour cent de masse de P au maximum, 0,08 pour cent de masse de Cu au maximum, 0,08 pour cent de masse de Al au maximum et aussi de 0,10 à 0,45 pour cent de masse de C, 1,2 à 2,5 pour cent de masse de Mn, de 1,2 à 2,5 pour cent de masse de Si avec le reste de Fe et très petits quantités des éléments de trace et contenant en priorité des éléments à micro-alliage Nb, V, Ti où les tuyaux sont produits par le tréfilage, l'extrusion, le laminage ou par la combinaison de ces procédés d'aciers à la microstructure de multiphase,
**caractérisée par** ce que le procédé de production se compose du traitement thermomécanique et/ou du traitement à chaude intercritique où les tuyaux sont produits par le laminage à chaude ou l'extrusion à chaude à température de formage finale entre 600 et 1000 °C
et par le refroidissement commandé suivant à retard de 50 sec au maximum en l'étendu de température de 700 à 450°C et à retard de 120 sec au minimum en l'étendue de température de 450 à 350°C.

2. Méthode de la production des tuyaux d'acier de haut rigidité et à basse alliage selon le revendication 1,
**caractérisée par** ce que le procédé du laminage à chaud ou l'extrusion à chaud est suivi par la séquence suivant : le procédé de refroidissement, le traitement intercritique à chaud à température maximal entre 720 et 850°C, à la compensation à cette température avant le pas du refroidissement commandé.

3. Méthode de la production des tuyaux d'acier de haut rigidité et à basse alliage selon le revendication 2,
**caractérisée par** ce que le procédé du laminage à chaud ou l'extrusion à chaud est suivi par le procédé de refroidissement et la fabrication est achevé par le tréfilage et/ou le formage par pression interne et/ou par le pliage.
